

Nov. 24, 1942.

A. H. BURKHOLDER

2,302,936

METHOD OF BLEACHING TEXTILE MATERIALS

Filed March 2, 1940

3 Sheets-Sheet 1



Nov. 24, 1942.

A. H. BURKHOLDER

2,302,936

METHOD OF BLEACHING TEXTILE MATERIALS

Filed March 2, 1940

3 Sheets-Sheet 2



Nov. 24, 1942.

A. H. BURKHOLDER

2,302,936

## METHOD OF BLEACHING TEXTILE MATERIALS

Filed March 2, 1940

3 Sheets-Sheet 3



FIG. 3



FIG. 4

Inventor  
ALDEN H. BURKHOLDER

Charles E. Nerrstrom

Attorney

## UNITED STATES PATENT OFFICE

2,302,936

## METHOD OF BLEACHING TEXTILE MATERIALS

Alden H. Burkholder, Cleveland, Ohio, assignor to  
 Industrial Rayon Corporation, Cleveland, Ohio,  
 a corporation of Delaware

Application March 2, 1940, Serial No. 321,934

6 Claims. (Cl. 8—108)

This invention relates to the bleaching of textile materials; more particularly, to methods of bleaching fibers, threads, fabrics or the like. Cotton and other materials of natural origin may be bleached according to the teachings of the invention, but it is in the bleaching of materials of regenerated cellulose that the invention may be employed to the greatest advantage. As herein-after explained, the invention is especially useful in the continuous processing of viscose artificial silk thread.

Textile materials are usually subjected, at some stage in the processing thereof, to the action of a bleaching agent, for the color of the unbleached material is objectionable for many uses. In the case of unbleached cellulose, the objectionable color is usually attributable to the presence of complex organic impurities many of which are eliminated or otherwise rendered innocuous by the use of bleaching agents which are known to have an oxidizing action. Such bleaching agents include not only chlorine but also solutions of potassium chlorite, sodium chlorite, sodium hypochlorite, sodium hypobromite, calcium hypochlorite or the like.

For a given material, the methods of application of the bleaching agent play an important part in the efficiency of the operation, but the bleaching power of the bleaching agent, and hence most of its efficiency, is dependent upon the amount of its "available chlorine." The latter factor is an arbitrary measure of its bleaching power, this even though the bleaching agent contains a substance other than chlorine as the principal bleaching constituent. Solutions of sodium hypochlorite, which are particularly effective in this respect, are widely used as bleaching agents; however, the other substances already mentioned may also be employed.

In general, the activity of a given bleaching solution may be regulated by varying such factors as its pH value, concentration, temperature, etc., as well as by controlling the length of time during which it is applied. Heretofore, it has been usual to maintain such bleaching solutions at a pH value substantially greater than 7; indeed, definite alkalinity has been thought to promote stability of the solution. The present invention, on the other hand, provides a method of bleaching pursuant to which the material to be bleached is subjected to treatment with a bleaching solution having a pH of substantially 7, preferably for a relatively short period of time.

The method of determining the pH of the

bleaching solution is more fully described herein-after.

Following bleaching operations carried out in the ordinary manner, it has been customary to treat the bleached material with an antichlor to arrest the action of any bleaching solution remaining therein; otherwise, such excess bleaching solution might continue to act upon the material to such an extent as to damage it. Notwithstanding the fact that it has long been desired to dispense with the use of an antichlor in order that the time and cost involved in applying it might be saved, its use has heretofore been regarded as inescapable. The present invention successfully eliminates the antichlor even under conditions in which its use has been considered to be indispensable.

The facility with which the present invention may be employed renders it particularly adaptable to the continuous processing of thread or the like. In such a process, it is desirable to process substantially continuous lengths of thread on apparatus generally similar to that shown, described and claimed in application Serial No. 25 7,114, filed February 18, 1935, by W. F. Knebusch and A. H. Burkholder (Patent 2,225,642). The invention provides a novel method of bleaching regenerated cellulose thread while it is continuously but temporarily stored in the form of an advancing helix characterized by a large number of closely spaced turns, the thread being treated while in this form with a bleaching solution containing a strong-acid-neutralized oxy-halogen salt of an alkali or alkaline-earth metal; the 30 thread is thereafter washed without the use of an antichlor and subsequently dried.

For convenience, the invention will be described as employed in continuous processing of multiple filament viscose artificial silk thread.

40 In the drawings, Figure 1 represents a vertical sectional elevation of one form of apparatus for the manufacture of viscose artificial silk thread by a continuous process in connection with which the present invention may be employed. Figure 45 2 is an end elevation of said apparatus showing the parts of the fluid circulating system with which the present invention is concerned, other parts being omitted for the sake of clearness. Figure 3 is a detail elevation, on an enlarged scale, 50 of a portion of the apparatus of Figure 2 for applying bleaching solution and a subsequent washing liquid to the thread, parts of the apparatus being broken away for the sake of clearness. Figure 4 represents a flow diagram of the path followed by the bleaching solution and washing

liquid as they are supplied to and withdrawn from the apparatus shown in Figure 3.

By referring to Figure 1, each thread 1 is formed by the extrusion of viscose through a spinneret 2 into a coagulating bath 3 contained in trough 4. After extrusion, the thread 1 is drawn vertically upward by and to a first thread-advancing reel 5 of a downwardly extending, catenate series of thread-advancing reels 5 to 14, inclusive, to each of which the thread passes in sequence. Each of said thread-advancing reels 5 to 14 is of cantilever construction, being adapted to advance the thread lengthwise thereof in a large number of closely spaced, generally helical turns. The thread 1 is discharged at the unsupported end of each reel, from which it passes to the succeeding reel.

The unsupported end of each reel 5 is disposed beyond the lateral edge of trough 4, thus enabling the thread 1 leaving the reel to pass vertically downward through channel 15 to the supported end of reel 6, the second reel of the series. The thread on reel 6 is not subjected to the action of any processing liquid other than coagulating liquid carried up to reel 5 by the thread leaving coagulating bath 3. The function of reel 5, in addition to drawing the thread from coagulating bath 3, is to provide a period for completion of coagulation of the thread; i. e., regeneration of the cellulose content thereof.

Means are provided for applying to the thread on reels 6 to 9, inclusive, processing liquids such as those for hardening, desulfurizing, washing, etc. Reels 10 and 11 have associated therewith means for bleaching and washing the thread according to the present invention, as more fully described hereinafter. On reel 12 a finishing liquid is applied to the thread. Reel 13 may be a drip reel on which the thread is stored for a period long enough to permit excess liquid to drip therefrom before it is passed to drying reel 14.

From reel 14 the dried thread passes directly to cap twister 16.

In the apparatus shown in the drawings, reels 5 to 14, inclusive, are disposed in stepped arrangement with their unsupported ends extending in the same direction and with the thread-receiving end of each reel in apposite relation to the thread-discharge end of the preceding reel. Corresponding reels in adjacent downwardly extending series are disposed in horizontal series lengthwise of the machine, so that the machine as a whole comprises two inclined banks of reels disposed on opposite sides of coagulating trough 4. The arrangement of reels in each bank and the arrangement of banks provide important advantages in making possible easy accessibility to the reels for operating purposes.

Each of reels 6 to 12, inclusive, has associated therewith a tube 17 by means of which liquid is applied to the thread. Each of said reels is tilted so that its thread-discharge end is elevated slightly. The liquid is applied toward the thread-discharge end of the reel in such manner that it forms a film which envelops the thread on the reel. The liquid dripping from the reel is collected in a trough 18 below the reel extending beneath adjacent reels in the same horizontal series.

Distributing tubes 17 for each of the liquid processing reels other than reel 6 are supplied with processing liquid from a conduit 19 formed integrally with the forward edge of collecting trough 18 disposed beneath the preceding reel. Each conduit 19 extends longitudinally of the

apparatus and supplies liquid to a plurality of corresponding reels disposed in the same horizontal series. Tubes 17 for reels 6 are supplied from a separate longitudinally extending conduit 21 disposed above reels 6.

Figures 2 to 4, inclusive, illustrate the system by which bleaching solution and wash water may be prepared and supplied to thread 1 according to the present invention.

In the preparation of a suitable sodium hypochlorite solution, water is supplied to reaction tank 25, shown diagrammatically in Figure 4, through a pipe 22. Sodium hydroxide solution; for example, a solution of approximately 19% NaOH, is supplied from reservoir 23 through pipe 24, the solution being diluted to the desired concentration (e. g., approximately 5% NaOH) with water from pipe 22. Chlorine from container 26 is supplied through pipe 27 to reaction tank 25, where it is passed through the diluted caustic solution to form sodium hypochlorite. The volume of water, caustic and chlorine passed to reaction tank 25 is preferably so regulated by valves 28 in the respective pipes 22, 24 and 27, that the reaction is carried to a point slightly on the alkaline side.

The desired concentration is reached when approximately 0.43% NaOH, calculated as free alkali, is left in the sodium hypochlorite solution, which preferably contains about 4% NaOCl.

The temperature of the solution in reaction tank 25 is maintained throughout the reaction at a moderate level, preferably about 19° C. This may conveniently be done by passing cooling brine from pipe 29 through a cooling jacket around reaction tank 25. If desired, however, water supply pipe 22 may be jacketed with a cooling medium to reduce the temperature of the water added to reaction tank 25 as a diluent, thereby obtaining a resultant low reaction temperature.

The prepared solution is withdrawn from reaction tank 25 through conduit 31 to make-up tank 32.

In the make-up tank, the excess alkali (approximately 0.43% NaOH) is neutralized by the addition of dilute hydrochloric acid from container 33 through conduit 34. The solution is adjusted to a pH of substantially 7 as determined by the use of Bromthymol Blue as an indicator after the available chlorine has been dissipated by the addition of hydrogen peroxide. Other acids, such as sulfuric, hydrobromic, phosphoric, etc., or even strong acid salts such as sodium acid sulfate, etc., may be employed to neutralize the free alkali, hydrochloric acid being given merely as an example.

The concentration of hypochlorite solution is then adjusted from approximately 4% NaOCl to approximately 0.05% NaOCl by the addition of warm water from water-heating tank 35 through pipe 36. Water may be supplied to tank 35 from the pipe 22 supplying reaction tank 25. The temperature of the water added to make-up tank 32 is preferably such that the resulting solution will be at a temperature of approximately 30° C. when applied to thread 1 on reel 10. To the liquid in make-up tank 32 is also added partially spent bleaching solution returned through conduit 37 as hereinafter explained.

The bleaching solution thus prepared passes from make-up tank 32 through conduit 38 to suitable temporary storage tanks 39 from which it may be withdrawn, as by means of pumps 41, as needed by constant-head supply box 43 (Fig-

ures 2 and 3). Constant-head supply box 43 furnishes bleaching solution through feed pipes 44 to conduits 18 for reels 10. Supply pipe 42, associated with pumps 41, preferably supplies more bleaching solution to constant-head supply box 43 than is passed therefrom through feed pipes 44; consequently, overflow 45 is provided in constant-head supply box 43 to permit the excess to escape through conduit 46. In this manner, the hydrostatic pressure in feed pipes 44, conduits 18, and distributor tubes 17 is maintained at a substantially constant value.

As shown in Figure 3, bleaching solution passed through feed pipes 44 and conduit 18 formed integrally with the forward edge of trough 18 below reels 10 is applied to the thread on each reel 10 through its corresponding distributor tube 17. The film of liquid which forms on reel 10 effects particularly efficient treatment of the thread before the partially spent liquid drips into trough 18. Where reel 10 is 5 inches in diameter, stores about 50 meters of thread thereon, and rotates at about 170 R. P. M., it is desirable to supply the bleaching solution through each of the distributor tubes 17 at the rate of approximately 250 c. c. per minute to obtain optimum results.

An aperture 47 at one end of each trough 18 permits the bleaching liquid collected thereby to be withdrawn by gravity from trough 18 through drain pipe 48 associated therewith. Conduit 48 communicating with drain pipes 48 and with conduit 46 from overflow portion 45 of constant-head supply box 43 conducts the bleaching solution into a trap 50, which has a partition 51 therein. In case of emergency, some of the liquid in trap 50 may pass over partition 51 in said trap, through pipe 52 to waste pipe 53, thence to a sewer. Ordinarily, however, the major portion of the solution from conduits 46 and 48 passes from trap 50 through return pipe 57 to make-up box 32.

Due to the character of the process, the bleaching solution applied to the thread in the system hereinabove described tends to become slightly acid during the progress of the bleaching operation. Consequently, when the partially spent bleaching solution is returned to make-up tank 32 through line 37, the acidity thereof is counteracted by the free alkali in the fresh hypochlorite solution added through pipe 31 from reaction container 25. The fresh hypochlorite solution thus added serves to refresh the supply of "available chlorine" in the bleaching solution.

Often the free alkali added with the fresh hypochlorite solution is greater than the amount necessary to neutralize the acidity of the partially spent solution. As a consequence thereof, it may be necessary to add more hydrochloric acid from container 33 and readjust the solution to a pH value of 7 as already described. Under certain circumstances, it may be necessary to add fresh caustic instead of acid to the spent solution to keep the desired pH value. In such case, caustic may be supplied directly from tank 23 through line 69 to make-up tank 32.

Inasmuch as it is desirable to refresh the bleaching solution continuously with the circulation thereof, it is usually found necessary to discard a measured volume of partially spent liquid per unit of time, as by bleeding off liquid from return pipe 37 through line 40. In this manner, the volume of continuously refreshed bleaching solution, allowing for addition of water, fresh bleaching solution, evaporation and other loss of

fluid, will be maintained substantially constant. The rate of discarding, and likewise the rate of addition of fresh bleaching solution, may be determined by the denier of the thread, the desired concentration of NaOCl, the temperature of the solution, etc.

The wash liquid supplied to the thread on reel 11, which may be fresh water, is conducted to reel 11 by means similar to those hereinabove disclosed in connection with the supply of bleaching solution to the thread on reel 10.

In the system illustrated, heated wash water from tank 35 is supplied by pumps 54, pipe 38 and supply pipe 55 to constant-head supply box 56. Feed pipes 57 conduct the water under substantially constant hydrostatic pressure from supply box 56 to conduits 18 formed in the forward edge of each trough 18 disposed below reels 10. The wash water is supplied from conduits 18 through distributor pipes 17 associated with reels 11. The water supplied to reels 11 from tank 35 is heated, as by steam coils, to a temperature such that the wash liquid prepared therefrom, when applied to thread 1, will have a temperature of approximately 30° C.

An overflow portion 58 is provided in constant-head supply box 56 by which excess water supplied through pipes 55 associated with pumps 54 may pass through overflow conduit 59 to wash water trap 60.

Water leaving the thread stored on reels 11 is collected in another trough 18 disposed therebelow. The contaminated water passes through aperture 61 in said trough 18 to drain pipes 61. A common conduit 62 communicating with the drain pipes 61 on opposite sides of the apparatus conducts the contaminated wash water to trap 60. If it is found to be desirable to reuse the commingled washing liquid, for instance, on another treating stage, it may be passed from trap 60 through pipe 63 to suitable recirculating means; otherwise, pipe 63 may communicate with the sewer. In case of emergency, liquid overflowing the partition 64 in trap 60 passes through pipe 65 to waste pipe 53 to be discarded.

Valves 67 in pipes 42 and 55 near supply boxes 43 and 56, respectively, serve to regulate the volume of liquid passed to said supply boxes.

In the continuous processing of thread, the bleaching solution is not stored for any long period but is constantly recirculated, so that no substantial decomposition of the bleaching solution tends to occur in spite of the neutralization of the free alkali with a strong acid. Thorough bleaching and washing of the thread is obtained even though the thread is subjected to each of these treatments for less than a minute. This results from the fact that a relatively high ratio of liquid to thread is provided, as well as from the fact that the operations are performed at moderate temperatures.

It has been found that under such circumstances, no treatment of the thread with an antichlor is required. It is only necessary that the thread be thoroughly washed, after which it may be dried or, as in the illustrated embodiment of the invention, be subjected to other processing treatment. Thread produced as above described is not uniformly bleached but is of high quality: despite the fact that no antichlor is applied thereto, its physical and physico-chemical characteristics are in no way impaired.

Besides making possible the omission of the anti-chlorination step, the invention has been

found to give rise to increased bleaching efficiency.

The foregoing description of the invention is illustrative merely: various modifications may be made therein without departing from the spirit of the invention. As hereinbefore indicated, other alkali or alkaline earth oxy-halogen bleaching solutions than sodium hypochlorite solutions may be used. Similarly, strong acid or strong acid salts other than hydrochloric acid may be used to neutralize the free alkali in the particular oxy-halogen solution employed. Other changes may be made within broad limits in the procedural aspects of the invention.

Numerous modifications may likewise be made in the apparatus; indeed, the invention may readily be practiced by means of sundry other types of processing apparatus. The invention is not restricted to the continuous processing of artificial silk thread, but may, under suitable conditions, be employed to process various other kinds of artificial threads. It may also be employed in the processing of many other textile materials, including those of natural origin.

It is intended that the patent shall cover, by suitable expression in the appended claims, whatever features of patentable novelty reside in the invention.

What is claimed is:

1. The method of bleaching regenerated cellulose thread comprising continuously but temporarily storing the thread in the form of an advancing helix characterized by a large number of closely spaced turns; treating the thread while in helical form with a bleaching solution containing a strong-acid-neutralized oxy-halogen salt of a metal from the group consisting of the alkali and alkaline-earth metals, said solution having an available chlorine content such that

the time required for bleaching the thread is less than a minute; washing the bleached thread without using an antichlor; and drying the washed thread.

5. 2. The method of bleaching regenerated cellulose thread comprising continuously but temporarily storing the thread in the form of an advancing helix characterized by a large number of closely spaced turns; treating the thread while in helical form with a bleaching solution containing a strong-acid-neutralized oxy-halogen salt of a metal from the group consisting of the alkali and alkaline-earth metals; washing the bleached thread while in helical form without using an antichlor, the washing time being less than a minute; and drying the washed thread.

3. The method of bleaching regenerated cellulose thread comprising continuously but temporarily storing the thread in the form of an advancing helix characterized by a large number of closely spaced turns; treating the thread while in helical form with a bleaching solution containing a strong-acid-neutralized oxy-halogen salt of a metal from the group consisting of the alkali and alkaline-earth metals, said solution having an available chlorine content such that the time required for bleaching the thread is less than a minute; washing the bleached thread while in helical form without using an antichlor, the washing time being less than a minute; and drying the washed thread.

4. The method set forth in claim 1 wherein the oxy-halogen salt is sodium hypochlorite.

5. The method set forth in claim 2 wherein the oxy-halogen salt is sodium hypochlorite.

6. The method set forth in claim 3 wherein the oxy-halogen salt is sodium hypochlorite.

ALDEN H. BURKHOLDER.

CERTIFICATE OF CORRECTION.

Patent No. 2,302,936.

November 24, 1942.

ALDEN H. BURKHOLDER.

It is hereby certified that error appears in the printed specification of the above numbered patent requiring correction as follows: Page 3, second column, line 70, for "not uniformly" read --not only uniformly--; and that the said Letters Patent should be read with this correction therein that the same may conform to the record of the case in the Patent Office.

Signed and sealed this 12th day of January, A. D. 1943.

Henry Van Arsdale,

Acting Commissioner of Patents.

(Seal)